

(No Model.)

J. T. EDSON.

FIBROUS PULP ROOFING TILE.

No. 310,192.

Patented Jan. 6, 1885.

Fig. 1.



Fig. 2.



WITNESSES

A. L. Lord  
John B. Hall

INVENTOR  
Julius T. Edson  
By Thos. B. Hall  
ATTORNEY

# UNITED STATES PATENT OFFICE.

JULIUS T. EDSON, OF CLEVELAND, OHIO, ASSIGNOR OF ONE-HALF TO  
HOWARD W. WHITE, OF SAME PLACE.

## FIBROUS-PULP ROOFING-TILE.

SPECIFICATION forming part of Letters Patent No. 310,192, dated January 6, 1885.

Application filed July 28, 1884. (No model.)

*To all whom it may concern:*

Be it known that I, JULIUS T. EDSON, a citizen of the United States, residing at Cleveland, county of Cuyahoga, and State of Ohio, have invented certain new and useful Improvements in Fibrous-Pulp Roofing-Tile; and I do hereby declare the following to be a description of the same and of the manner of constructing and using the invention in such full, clear, concise, and exact terms as to enable any person skilled in the art to which it appertains to construct and use the same, reference being had to the accompanying drawings, forming a part of the specification, the principle of the invention being herein explained and the best mode in which I have contemplated applying that principle, so as to distinguish it from other inventions.

My invention is that of the manufacture of a roofing-tile formed by passing fibrous pulp through certain processes, hereinafter stated and described. The article thus produced is impervious to water, resists heat, is not brittle or frangible like slate, is not affected by the frosts and ice of winter, is as easily handled and nailed as shingles, and presents a finished and attractive appearance. It also may very readily be cut and shaped into any desired form and size.

In the drawings, Figure 1 is a plan view of a tile. Fig. 2 is a vertical cross-section of the same, A showing the body of the pulp, and B and C outer coatings, as hereinafter specified.

The process of the manufacture of this tile is as follows: Any available and suitable fibrous pulp being prepared, portions of it are pressed, by any means or machinery, into such forms as are desired. These forms, being sufficiently dried, are then subjected to a water-proof solution until they are thoroughly impregnated therewith. They are then sufficiently baked to harden in them the material constituents received from said solution. After this baking the articles are treated with a mixture that imparts to them an enameled surface, adapting them to resist the action of heat. Before this enamel has entirely hardened, while it is yet sticky, a coating of sand is applied to it, which adds to its adaptability to endure heat and resist flame. Said sand being thus applied, the tiles are still again

subjected to a baking heat. Said sand is indicated by C in Fig. 2, and said enamel is indicated by B in same figure.

By the use of varied-colored sand a variety of colors may be given to the tile.

Of the tile thus produced its advantages for roofing purposes over and above those of slate are many. In a slate roof great weight is absolutely unavoidable, while the pulp tile is very light, obviating the necessity of the heavy roof-frame requisite for a slate roofing. From the inherent brittleness of a slate tile it is constantly liable to be broken from the blow of stones or other articles upon it, or from human footsteps, while the pulp tile, prepared as herein set forth, is devoid of such imminent frangibility. Also, as water works into the joints and under the layers of a slate roof and freezes, there is great exposure to a breaking. Also, it is impracticable to have slate tiles lie compactly together on a roof, their brittle nature not permitting them to be very tightly drawn together by the nails. Also, the drilled holes of slate tiles expose them to some lateral motion. All such deficiencies are obviated by the herein-described pulp tile. In the present invention the nails may be driven as close home as they are in shingles, so as to bind and bed the tiles most completely together without the possibility of any lateral movement. Nails penetrate them with greater ease than they do shingles, and are hugged closer by the elastic quality of the pulp than by the more rigid quality of wood.

And to these advantages must be added the cheapness of the pulp tile above one of slate and the ease of its transportation. Also, my invention is not confined to roofing, but may be readily applied to other uses, as of interior decoration, as of walls, or otherwise. It affords a fabric of feasible application to any surface, and furnishes a handsome and attractive appearance. When left without the applied sand, the enamel gives a bright and lustrous surface, peculiarly fitting it for indoor uses or other similar applications.

What, therefore, I claim is—

1. A fibrous-pulp tile impregnated with a water-proof solution and enameled with a fire-proof solution, substantially as set forth.
2. A fibrous-pulp tile impregnated with a

water-proof solution, enameled with a fire-proof solution, and provided with a coating of sand, substantially as set forth.

3. A process of making fibrous-pulp tile by, first, pressing the pulp into the desired form; second, drying the same; third, impregnating said tile with a water-proof solution; fourth, subjecting said tile to a baking heat; fifth, treating said tile with a fire-proof solution; sixth, furnishing said tile with a coating

of sand; and, seventh, subjecting said tile to another operation of baking heat, substantially as set forth.

In testimony that I claim the foregoing to be my invention I have hereunto set my hand this 24th day of July, A. D. 1884.

JULIUS T. EDSON.

Witnesses:

J. B. FAY,

JNO. G. HALL.